

## UNITED STATES PATENT OFFICE

OTTO MATTHIES AND BRUNO WENDT, OF DESSAU IN ANHALT, GERMANY, ASSIGNEES  
TO AGFA ANSCO CORPORATION, OF BINGHAMTON, NEW YORK, A CORPORATION OF  
NEW YORK.

LIGHT-SENSITIVE SILVER HALIDE EMULSIONS AND PROCESS OF MANUFACTURING  
THE SAME

No Drawing. Application filed January 28, 1929, Serial No. 335,733, and in Germany January 31, 1928.

The present invention relates to photographic silver salt emulsions of increased stability, little tendency to fog and determined grain size, to layers containing the same and to a process for manufacturing the same.

We found that all organic nitrogen compounds with three or more nitrogen atoms in the molecule containing at least one  $=\text{NH}$  group, the H atom of which is liable to substitution by silver, thus forming stable silver salts the solubility of which is approximately of the same range as that of silver chloride, are able to increase the stability and lessen the tendency to fog of light sensitive silver halide emulsions on being added to the finished emulsion or to any of its constituents during manufacture. The compounds which form silver salts of the least solubility exert the strongest effect on the stability of emulsions.

It has furthermore been found that the said compounds when present during the addition of the silver nitrate solution restrain the growing of silver bromide grains and thus give to the emulsion a steeper gradation while in the same time increasing its stability.

By our present process we may thus obtain emulsions of varying steepness of gradation though starting with the same proportions of constituents. The said addition may be made to the finished emulsion or to its constituents at any stage of its manufacture or of emulsion making.

The following examples illustrate the invention:

*Example 1.*—In a prescription for the manufacture of a highly sensitive negative-emulsion with use of a gelatine which produces fog, there is added to the gelatine, while it is being digested, 50 milligrams of tetrazole per 100 grams of silver nitrate. There is obtained a highly sensitive, clear emulsion.

*Example 2.*—A highly sensitive negative emulsion is made according to any known prescription and before the silver salt solution is run into the potassium bromide solution there are added to the latter 70 milligrams of 5-methylbenzotriazole per each 100 grams of silver nitrate. There is thus ob-

tained a clear emulsion of finer grain than when made without the addition of 5-methylbenzotriazole.

We claim:

1. A process of manufacturing light sensitive silver halide emulsions of increased stability, in which there is added to the emulsion a compound forming a stable silver salt of no higher solubility than silver chloride and containing at least 3 nitrogen atoms in the molecule at least one of which being linked to a hydrogen atom which is liable to substitution by silver. 55

2. A process of manufacturing light sensitive silver halide emulsions of increased stability, in which there is added to a constituent of the emulsion at any stage of the manufacture a compound forming a stable silver salt of no higher solubility than silver chloride and containing at least 3 nitrogen atoms in the molecule at least one of which being linked to a hydrogen atom which is liable to substitution by silver. 65

3. A process of manufacturing light sensitive silver halide emulsions of increased stability and restrained size of silver halide grains, in which there is added to a constituent of the emulsion prior to the addition of silver nitrate a compound forming a stable silver salt of no higher solubility than silver chloride and containing at least 3 nitrogen atoms in the molecule at least one of which being linked to a hydrogen atom which is liable to substitution by silver. 75

4. A process of manufacturing light sensitive silver halide emulsions of increased stability, in which there is added to the emulsion a compound forming a stable silver salt of no higher solubility than silver chloride and containing 3 nitrogen atoms in the molecule at least one of which being linked to a hydrogen atom which is liable to substitution by silver. 80

5. A process of manufacturing light sensitive silver halide emulsions of increased stability, in which there is added to a constituent of the emulsion at any stage of the manufacture a compound forming a stable silver salt of no higher solubility than silver chloride and containing 3 nitrogen atoms in 90

the molecule at least one of which being linked to a hydrogen atom which is liable to substitution by silver.

6. A process of manufacturing light sensitive silver halide emulsions of increased stability and restrained size of silver grains, in which there is added to a constituent of the emulsion prior to the addition of silver nitrate a compound forming a stable silver salt of no higher solubility than silver chloride and containing 3 nitrogen atoms in the molecule at least one of which being linked to a hydrogen atom which is liable to substitution by silver.
- 10 7. Light sensitive silver halide emulsions containing a compound forming a stable silver salt of no higher solubility than silver chloride and containing at least 3 nitrogen atoms in the molecule at least one of which being linked to a hydrogen atom which is liable to substitution by silver.
- 15 8. Light sensitive silver halide emulsions containing a compound forming a stable silver salt of no higher solubility than silver chloride and containing 3 nitrogen atoms in the molecule at least one of which being linked to a hydrogen atom which is liable to substitution by silver.
- 20 9. A process of manufacturing light sensitive silver halide emulsions of increased stability comprising the step of adding tetrazole.
- 25 10. A process of manufacturing light sensitive silver halide emulsions of increased stability comprising the step of adding tetrazole to a constituent of the emulsion at any stage of its manufacture.
- 30 11. Light sensitive silver halide emulsions containing tetrazole.
- 35 12. Light sensitive silver halide emulsions containing tetrazole added to a constituent of the emulsion at any stage of its manufacture.

In testimony whereof, we affix our signatures.

45 OTTO MATTHIES.  
BRUNO WENDT.